

# United States Patent Office

3,720,549

Patented Mar. 13, 1973

1

3,720,549

3,726,349

**INSULATING COATING AND METHOD OF  
MAKING THE SAME**

MAKING THE SAME  
Robert G. Hirst and George J. Desnoyers, Pittsfield,  
Mass., assignors to General Electric Company  
No Drawing. Filed Sept. 23, 1970, Ser. No. 74,508  
Int. Cl. C23f 7/26

U.S. Cl. 142—6.16

### 3 Claims

## ABSTRACT OF THE DISCLOSURE

Electrically insulating coating for strand annealed magnetic silicon steel is composed of an aqueous mixture of (1) the reaction product of chromium trioxide, formic acid and phosphoric acid, (2) phosphoric acid, and (3) colloidal silica.

The present invention relates to coated magnetic sheet material and a method of making the same. More particularly, the invention concerns refractory coating material which is applied to such sheet material, and especially to strand annealed silicon steel strip, and serves as a permanent insulating coating in the use of the metallic sheet material in laminated electrical structures.

The forms of magnetic sheet material with which the invention is concerned include strip material such as used in wound transformer cores, and cut or punched laminations forming stacked transformer cores or other electrical apparatus. Examples of compositions of magnetic sheet materials which may be effectively coated in accordance with the invention are silicon steel (typically containing about 1-5% silicon), nickel-iron alloys, common iron, and other ferromagnetic materials.

The invention is particularly applicable to silicon steel strip which has been subjected to a grain growth and purification anneal treatment wherein the steel is heated in the form of a single strand, as distinguished from coiled or stacked form, in a suitable furnace through which the strand may be continuously passed during the heat treatment.

In the past, it has been the practice to subject the steel sheet material in coiled or stacked form to the annealing treatment, and in order to prevent sticking of the sheet surfaces to each other during such elevated heat treatment, an insulating coating material such as magnesium hydroxide has conventionally been applied to the sheet material prior to such annealing stage. Such coating material has served both to avoid the problem of sticking during the anneal and to provide electrical insulation to reduce eddy current loss in the laminated core formed by the sheet material in its use in a transformer, motor or the like. However, the application of insulating coatings in general to the steel sheet prior to the annealing treatment has the disadvantage in a strand anneal procedure that the presence of the insulating coating tends to delay the purification of the steel during the strand anneal, e.g., by hindering removal of sulfur from the steel, and consequently the strand anneal process is not as rapid as it might be in the absence of such coatings. Moreover, the prior types of inorganic insulating coating such as magnesium hydroxide require relatively high curing temperatures, e.g., over 1000° C., to produce final coatings of the requisite hardness, electrical insulating and other properties. While such elevated tem-

2

peratures are employed during the usual grain growth and purification anneal, it has in many cases been found desirable to apply one or more additional insulating layers after the usual anneal and for this purpose the sheet material has to be heated again to elevated temperature to cure the added insulating layer.

It is, therefore, an object of the invention to provide an improved insulating material for metallic sheet material which avoids the above-mentioned disadvantages.

A further object of the invention is to provide an improved insulating coating composition for the above purposes which may be cured at relatively low temperatures.

Still another object of the invention is to provide an insulating coating composition which is particularly adapted for use on electrical steel sheet material treated by a strand anneal process.

It is another object of the invention to provide an improved method of making insulated steel sheet material of the above type.

Other objects and advantages will become apparent from the following description and the appended claims.

With the above objects in view, the present invention in one of its aspects relates to an insulating coating composition comprising a mixture of trivalent chromium, phosphoric acid, a finely divided refractory material selected from the group consisting of colloidal silica and colloidal alumina, and water. In a preferred embodiment of the invention, the trivalent chromium is obtained by reacting chromium trioxide and a reducing agent such as formic acid in phosphoric acid solution.

In a typical application of the present invention, the foregoing insulating mixture is deposited on the surfaces of silicon steel strip which has been subjected to a strand anneal process for producing the desired magnetic texture and removing undesired impurities therein. Such a strand anneal process is disclosed in detail, for example, in Fitz et al. Patent 2,986,485, and the disclosure of that patent is incorporated herein by reference. As there disclosed, the strand anneal process, which may be carried out on a continuous basis, comprises the steps of heating silicon steel material for about 5 to 60 minutes (preferably about 15 minutes) at a temperature of about 950 to 1050° C., and thereafter heating the material at a temperature of 1175 to 1250° C. for about 1 to 30 minutes (preferably about 15 minutes). The annealing treatment is preferably carried out in a reducing atmosphere in the furnace, such as in hydrogen or other reducing gases. In accordance with the invention, the thus annealed steel strip, which previous to the anneal had not been provided with an insulating coating, is then coated with the above-described mixture, and the latter is then dried by heating or otherwise cured to form a hard, tightly adherent, highly insulating coating on the steel surfaces.

A particular mixture found eminently satisfactory for preparing the coating in accordance with the invention has the following composition, shown in a preferred and a range of proportions in percent by weight:

|                                                      | Preferred,<br>percent | Range,<br>percent |
|------------------------------------------------------|-----------------------|-------------------|
| Chromium trioxide-CrO <sub>3</sub> -----             | 2.2                   | 1-10              |
| Formic acid-HCOOH-----                               | 1.5                   | 1-10              |
| Phosphoric acid-H <sub>3</sub> PO <sub>4</sub> ----- | 18.8                  | 10-50             |
| Colloidal silica-----                                | 31.6                  | 15-50             |
| 65 Water-----                                        | 45.9                  | Balance           |

As a result of the reaction whereby the formic acid reduces the six-valent chromium of the chromium trioxide to trivalent chromium in phosphoric acid solution, the following compositions are ultimately obtained from the above compositions:

|                                                | Preferred, percent | Range, percent |
|------------------------------------------------|--------------------|----------------|
| Cr <sup>+++</sup> (as chromium phosphate)..... | 3.2                | 1-15           |
| Phosphoric acid.....                           | 16.9               | 10-40          |
| Colloidal silica.....                          | 32.1               | 15-50          |
| Water.....                                     | 47.8               | Balance        |

In an illustrative method which may be used in practicing the invention, the chromium trioxide in flake form is dissolved in water to form an orange colored solution. Phosphoric acid is added to this solution. Formic acid is then slowly added to the solution with stirring, producing a vigorous reaction with the evolution of CO<sub>2</sub> gas from the solution. An aqueous solution of chromium phosphate providing Cr<sup>+++</sup> ions (trivalent chromium) is thus produced in accordance with the following reaction:



As is evident the formic acid reduces the six-valent chromium in the chromium trioxide to produce the trivalent Cr<sup>+++</sup> ion.

After the thus obtained solution is diluted with the required amount of water, colloidal silica in the proportion shown above is mixed with the solution.

The mixture thus produced is a green liquid having a specific gravity of 1.19 and a pH of about 1.6. The coating solution is applied to the strand annealed steel material in any suitable manner such as by rolling, dipping, spraying, brushing or other methods. Typically, the steel strip, which has been allowed to cool to room temperature, is passed over rollers for applying the coating and then baked in an oven at about 300° C. for about 1 minute.

The coating thus produced was smooth, hard and tightly adherent and did not craze appreciably on bending of the coated sheet material. It was characterized by excellent electrical insulation properties, had minimal effect on watt-loss and permeability properties. It was found by test, for example, that such a coating deposited in an amount of .05 oz./sq. ft. on the steel sheet provides a Franklin insulation value of about 0.0-0.1 ampere, it being known by those skilled in the art that any Franklin value below .20 ampere is satisfactory for transformer use, and that the lower this value the better the insulating quality.

The colloidal silica which may be used in the described mixture is in the form of an aqueous suspension containing SiO<sub>2</sub> in an extremely finely divided form made by an ion exchange technique. Colloidal silica is available commercially under the trade mark of Ludox, a product of E. I. du Pont de Nemours & Company, which is an aqueous colloidal sol containing approximately 30% SiO<sub>2</sub> with less than 0.5% Na<sub>2</sub>O as a stabilizer. A more detailed description of this colloidal silica is found in Robinson Patent 2,809,137, which description is incorporated herein by reference.

As an alternative to the colloidal silica there may be used colloidal alumina, which is a dispersion in water of alumina particles which are sufficiently finely divided to provide a colloidal sol in water. A colloidal form of alumina available commercially which may be used is sold under the trademark Baymal, a product of E. I. du Pont de Nemours & Company. This is a white, free-flowing powder consisting of minute fibrils of boehmite (AlOOH) alumina and which disperses readily in water to yield a colloidal sol. Further detailed descriptions of this material and colloidal sols thereof and methods of making them

are set forth in the patent to Bugosh 2,915,475. In general, for the purposes of this invention a concentration of 5-50 grams per liter of water of the finely divided colloidal alumina has been found suitable, with a range of 30-40 grams/liter affording optimum results.

5 Finely divided refractory materials other than those described above may also be found useful.

Although the temperature used for drying the coating as described above is preferred, the drying stage temperature may vary in a range of about 200° C. for 3 minutes to about 400° C. for about 1/2 minute.

10 The composition of the finally produced coating, which is transparent and pale green in color, is not presently known and cannot be definitely ascertained, and it is accordingly referred to herein simply as the cured product of the mixture of ingredients as above described.

15 While formic acid was proved particularly satisfactory as a reducing agent for use in the above mixture, other reducing agents may be used provided that they do not include contaminating ions which are harmful to the insulating properties of the coating or the dielectric liquid of the transformer or other apparatus in which the coated steel is used. Examples of other suitable reducing agents which may be found useful are oxalic acid, phosphorous acid and hypophosphorous acid.

20 It should be understood that while the described insulating coating is particularly applicable for use on strand annealed silicon steel material, it is not limited to such use. It will be found of advantage, for example, for coating such steel or other metallic material where relatively low curing temperatures are or must be used.

25 There is thus provided in accordance with the invention an improved insulating coating composition which has excellent electrical insulating properties, may be deposited in thin and tightly adherent layers to the steel surface, which does not contribute to electrical losses or other unfavorable electrical properties in the coated steel material, and which is applied easily in a continuous operation. The very tenacious adherence of the insulating coating is 30 especially noteworthy in view of the very smooth surfaces which characterize strand annealed steel, as distinguished from steel annealed in coiled or stacked form as in conventional processes, and which ordinarily make it difficult for conventional insulating coatings to firmly adhere thereto.

35 40 45 While the present invention has been described with reference to particular embodiments thereof, it will be understood that numerous modifications may be made by those skilled in the art without actually departing from the scope of the invention. Therefore, the appended claims are intended to cover all such equivalent variations as come within the true spirit and scope of the invention.

50 55 What we claim as new and desire to secure by Letters Patent of the United States is:

1. An insulating coating composition comprising an aqueous mixture of (1) the reaction product of chromium trioxide, a reducing agent therefor for reducing the six-valent chromium to trivalent chromium, and phosphoric acid, (2) phosphoric acid, and (3) a finely divided refractory material, said reducing agent being selected from the group consisting of formic acid, oxalic acid, phosphorous acid and hypophosphorous acid, and said refractory material being selected from the group consisting of colloidal silica and colloidal alumina, said mixture comprising in percent by weight 1-10% chromium trioxide, 1-10% reducing agent, 10-40% phosphoric acid, 15-50% refractory material and the balance water.

60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 893

3,720,549

5

as defined in claim 1, and heating the same at a temperature of between 200° C. and 400° C.

6

2,768,104 10/1956 Schuster et al. ----- 148—6.16  
3,207,636 9/1965 Wada et al. ----- 148—6.16

References Cited

UNITED STATES PATENTS

3,562,011 2/1971 Hirst et al. ----- 148—6.16 X  
3,421,949 1/1969 Halversen ----- 117—135.1 X  
3,094,441 6/1963 Curtin ----- 148—6.16  
3,331,713 6/1967 Miller ----- 148—113  
3,030,601 2/1936 McDonald ----- 148—6.16 10 148—113

OTHER REFERENCES

5 Japanese Patent Publication No. SH043-7849, Mar. 26,  
1968.

RALPH S. KENDALL, Primary Examiner

U.S. Cl. X.R.